

# UNITED STATES PATENT OFFICE.

ARRIGO TEDESCO, OF TURIN, ITALY.

## METHOD FOR MANUFACTURING ALUMINIUM ALLOYS.

1,318,702.

Specification of Letters Patent. Patented Oct. 14, 1919.

No Drawing.

Application filed July 11, 1919. Serial No. 310,261.

To all whom it may concern:  
Be it known that I, ARRIGO TEDESCO, a subject of the King of Italy, and resident of Turin, Italy, have invented certain new and useful Methods for Manufacturing Aluminium Alloys, of which the following is a specification.

The methods usually employed in foundry work are such that it is difficult to obtain aluminium alloys of high strength and desirable mechanical characteristics; and above all, it has often been found that such alloys lack homogeneity.

The present invention relates to a method by means of which the association of aluminium with the other metals intended to enter into the final alloy, such as zinc, copper, titanium, and vanadium, is obtained in the best possible conditions, and particularly with a view to obtaining a properly homogeneous alloy.

The method according to this invention consists in preparing separately a bath of basis alloy containing a portion of from 10% to 20% of the total weight of the final alloy, said bath containing light metals to an amount of from  $\frac{1}{2}$  to  $\frac{2}{3}$  by weight relatively to the heavy metals.

A molten mixture is then made of the remaining metals of the final alloy, and a portion of from  $\frac{1}{2}$  to  $\frac{1}{2}$  said mixture is added to the basis bath while it is slightly overheated and is continuously stirred with an up-and-down motion.

When the portion of from  $\frac{1}{2}$  to  $\frac{1}{2}$  of the aforesaid second mixture has been added to the basis bath, the molten material thus obtained is poured into a crucible containing the metals of the final alloy not included in the basis bath or the second mixture.

By way of example, it being desired to produce an alloy having the following composition:

|                |       |
|----------------|-------|
| 45 Zinc-----   | 15.00 |
| Titanium-----  | 0.56  |
| Aluminium----- | 84.44 |

10 to 20 kg. of an alloy containing aluminium to about  $\frac{2}{3}$  kg. to each kg. of mixture 50 of zinc and titanium and the remainder of aluminium, zinc and titanium are melted separately. The first or basis bath containing  $\frac{2}{3}$  of aluminium is slightly overheated, and  $\frac{1}{2}$  to  $\frac{1}{2}$  of the second mixture is added

thereto, a continuous stirring being effected. 5 The material thus obtained is poured into the residuum of the second mixture, this method providing a thoroughly homogeneous alloy having the best possible mechanical characteristics. 60

What I claim as my invention and desire to secure by United States Letters Patent is:

1. A method for manufacturing aluminium alloys consisting in preparing a separate basis bath comprising a portion of the alloy constituents, overheating and stirring the same, making a mixture of the remainder of said constituents, adding a portion of this mixture to said basis bath while overheated and stirred, and pouring the material obtained into the residuum of said second mixture. 70

2. A method for manufacturing aluminium alloys consisting in preparing a separate basis bath comprising a portion of the alloy constituents, light metals being contained in this bath to a relative amount of  $\frac{1}{2}$  to  $\frac{2}{3}$  with regard to heavy metals, overheating and stirring the bath, making a mixture of the remainder of said constituents, 75 adding a portion of this mixture to said basis bath while overheated and stirred and pouring the material obtained into the residuum of said second mixture. 80

3. A method for manufacturing aluminium alloys consisting in preparing a separate basis bath comprising a portion of the alloy constituents, overheating and stirring the same, making a mixture of the remainder of said constituents, adding a portion from  $\frac{1}{2}$  to  $\frac{1}{2}$  of this mixture to said basis bath while overheated and stirred, and pouring the material obtained into the residuum of said second mixture. 85

4. A method for manufacturing alloys 95 consisting in preparing a separate basis bath comprising a portion of the alloy constituents, light metals being contained in this bath to a relative amount of  $\frac{1}{2}$  to  $\frac{2}{3}$  with regard to heavy metals, overheating and stirring the bath, making a mixture of the remainder of said constituents, adding a portion from  $\frac{1}{2}$  to  $\frac{1}{2}$  of this mixture to said basis bath while overheated and stirred and pouring the material obtained into the residuum of said second mixture. 100

Signed at Turin, Italy, June 12, 1919.  
ARRIGO TEDESCO.